# EUROPEAN PATENT SPECIFICATION

(11) **EP 2 992 120 B1**
(45) Date of publication and mention of the grant of the patent: **01.03.2017**
(21) Application number: 14721956.2
(22) Date of filing: 02.05.2014
(51) Int. Cl.: C22C 19/05

(54) **ALLOY COMPOSITION**
LEGIERUNGSZUSAMMENSETZUNG
COMPOSITION D'ALLIAGE

(30) Priority: 03.05.2013 GB 201308070
(43) Date of publication of application: 09.03.2016
(73) Proprietor: Goodwin Plc, Hanley Stoke-on-Trent ST1 3NR (GB)
(72) Inventor: ROBERTS, Stephen, Stone Staffordshire ST15 8YH (GB); THOMSON, Rachel, Clare, Loughborough Leicestershire LE11 2DH (GB); YANG, Yujin, Loughborough Leicestershire LE11 2NW (GB); LEESE, Ryan, Stoke-on-Trent Staffordshire ST4 8YE (GB)
(74) Representative: Jackson, Martin Peter
(86) International application number: PCT/GB2014/051384
(87) International publication number: WO 2014/177892

(56) References cited:
- FR-E- 55 100
- US-A- 4 461 659
- J M SANDERS ET AL: "Elimination of Fissures in Thick Section INCONEL Alloy 740 Welds", TECHNICAL PAPER BR-1827 BABCOCK & WILCOX POWER GENERATION GROUP INC., 31 May 2009 (2009-05-31), - 4 June 2009 (2009-06-04), XP055122574, USA
- SHAILESH J. PATEL ET AL: "Nickel Base Superalloys for Next Generation Coal Fired AUSC Power Plants", PROCEDIA ENGINEERING, vol. 55, 1 January 2013 (2013-01-01), pages 246-252, XP055122303, ISSN: 1877-7058, DOI: 10.1016/j.proeng.2013.03.250
- R. VISWANATHAN ET AL: "U.S. Program on Materials Technology for Ultra-Supercritical Coal Power Plants", JOURNAL OF MATERIALS ENGINEERING AND PERFORMANCE, vol. 14, no. 3, 1 June 2005 (2005-06-01), pages 281-292, XP055122191, ISSN: 1059-9495, DOI: 10.1361/10599490524039
- D.L. KLARSTROM ET AL: "Nickel-Base Alloy Solutions for Ultrasupercritical Steam Power Plants", PROCEDIA ENGINEERING, vol. 55, 1 January 2013 (2013-01-01), pages 221-225, XP055122305, ISSN: 1877-7058, DOI: 10.1016/j.proeng.2013.03.246
- K. MAILE: "Qualification of Ni-Based Alloys for Advanced Ultra Supercritical Plants", PROCEDIA ENGINEERING, vol. 55, 1 January 2013 (2013-01-01), pages 214-220, XP055122308, ISSN: 1877-7058, DOI: 10.1016/j.proeng.2013.03.245

## Description

The present invention relates to an alloy composition, in particular to a nickel base alloy composition. The alloy composition of the present invention is particularly suited for forming products by way of casting, as opposed to a wrought process (i.e. worked, forged or hammered etc.). The alloy of the present invention is suitable for use in high pressure steam turbine applications, amongst others; for example, use in a power station.

The drive for reduced carbon dioxide emissions and improved efficiency in coal fire power plants, has lead to much work being carried out around the world in regards to material development enabling a 700°C+ steam temperature operation with pressure of up to 80MPa or as high as 100MPa. At these elevated temperatures and pressures, steels do not have enough strength, so instead material development has focused on Nickel alloys.

Nickel alloy development in general has concentrated on two main groups of alloys, solution strengthened and precipitation strengthened alloys. The solid solution alloys are lower in strength than their precipitation hardened counter parts, and so have reduced stress rupture strength, but possess good ductility and weldability. Precipitation strengthened alloys have been used in jet engines.

Accordingly, the present invention seeks to provide a new alloy composition. In particular, the present invention seeks to provide a castable alloy composition with the required stress rupture strength for power plant operation above 700°C , and possibly even above 750°C.

Accordingly, the present invention provides an alloy consisting of, in mass %, 24.0-26.0% Cr, 19.0-22.0% Co, 1.00-1.60% Al, 1.00-1.60% Ti, up to 1.50% Fe, up to 0.020% C, up to 0.40% Si, up to 0.50% Mn, up to 0.50% Cu, up to 0.50% Mo, up to 0.50% Nb, up to 0.005% B, up to 0.03% Zr, up to 0.10% V, up to 0.02% Mg, up to 0.25% Ta, up to 0.010% S, up to 0.015% P, up to 0.20% W, up to 0.02% Ca, up to 0.05% N, up to 80 ppm Zn, up to 60 ppm Sn, up to 20 ppm Pb, and the balance Ni plus impurities.

The alloy of the present invention is precipitation strengthened and therefore has a higher stress rupture strength than previously used solid solution strengthened nickel alloys. Additionally, the alloy composition is castable.

The present invention will be more fully described by way of example with reference to the accompanying drawings in which:
- Figure 1 is a graph showing the relative stress rupture strength vs temperature of various steels and Ni Alloys for operation from 550°C to 760°C. The nickel alloys included in the graph are put forward as potential alloys for plant operation above 700°C;
- Figure 2 is a SEM micrograph showing cracking in a cast alloy after heat treatment;
- Figure 3 is an equilibrium phase diagram showing the phases present in the alloy of Figure 2;
- Figure 4 is an equilibrium phase diagram showing the MX, Eta and the M₂₃C₆ phases in the alloy of Figure 2;
- Figure 5 is an equilibrium phase diagram showing the phases present in an alloy of the present invention;
- Figure 6 shows the composition of MX of an alloy according to the present invention;
- Figure 7 is an equilibrium phase diagram showing Gamma Prime % versus Niobium concentration;
- Figure 8 is an equilibrium phase diagram showing Nb MX % versus Carbon content;
- Figure 9 is an equilibrium phase diagram showing the combined effect of Nb and C on Nb MX content;
- Figures 10-13 are equilibrium phase diagrams showing MX predictions for a range of carbon contents with fixed Nb at 0.25%;
- Figure 14 is a Scheil calculation for alloy 740;
- Figure 15 shows the effect of Tantalum on gamma prime (γ') mass %;
- Figure 16 shows the predicted beneficial effect of Mo on gamma prime (γ') mass %;
- Figure 17 is a bar chart comparing the room temperature tensile strength of the alloy of the invention with other cast candidate Ni alloys for Advanced Ultra Critical (A-USC) application
- Figure 18 is a bar chart comparing the room temperature yield strength of the alloy of the invention with other cast candidate Ni alloys for A-USC application;
- Figure 19 is a chart comparing the room temperature elongation and reduction in area of the alloy of the invention with alloy 263;
- Figure 20 is a graph of Stress Rupture Strength plotted against Larsen Miller Parameter of the Inventive Alloys (G130 & G130B) compared with public domain data for other candidate cast A-USC Ni Alloys; and
- Figure 21 is a graph of stress rupture strength plotted against Larsen Miller parameter of G130 & G130B for different section sizes;
- Figure 22 is a SEM micrograph showing G130B cast alloy after heat treatment; with no MX cracking observed.

In seeking to find an alloy composition with a high stress rupture strength at temperatures above 700°C (for example, a high pressure steam turbine casing, valve or (ancillary) valve components for a power plant) and which can be formed into a product by casting, the present inventors considered the Ni alloys shown in Table 1.

**Table 1: Typical Chemical Composition of 700°C + Candidate Alloys**

| Material Grade | Ni | Cr | Mo | Nb | Co | W | Al | Ti | Strengthening Mechanism | Other |
|---|---|---|---|---|---|---|---|---|---|---|
| Alloy 625 | BAL | 20 | 9 | 3.5 | - | - | 0.2 | 0.2 | SS | - |
| Alloy 263 | BAL | 20 | 6 | - | 20 | - | 0.6 | 2.4 | PH | Cu:0.20 |
| Alloy 230 | BAL | 22 | 2 | - | 5 | 14 | 0.3 | - | SS | B:0.015 |
| Alloy 617 | BAL | 22 | 9 | - | 12 | - | 1 | 0.5 | SS + PH | B:0.006 |
| Inconel ®740 | BAL | 25 | - | 2 | 20 | - | 1 | 1.8 | PH | B:0.003 |
| Haynes® 282® | BAL | 20 | 8.5 | - | 10 | - | 1.5 | 2.1 | PH | B:0.005 |

These alloys are strengthened either by a solid solution strengthening mechanism (SS) or by precipitation hardening (PH). These mechanisms are described briefly below.

Solid solution strengthened Ni alloys consist of an *fcc* matrix which is strengthened by the addition of solid solution strengtheners such as Mo, Cr, Co and W. This method of hardening depends upon the difference in lattice parameters between the Ni based austenitic structure and the solute atoms, the strengthening potency being proportional to this difference. The greater the percentage of solute atoms the greater will be the hardening effect. However, the amount of alloying additions is limited by the possibility of σ-phase formation and its accompanying disadvantages.

Precipitation hardening is accomplished in Ni alloys by the formation of three types of precipitate, gamma prime (γ') gamma prime prime (γ") (*or gamma double prime*)*,* and grain boundary borides and carbides. γ' is generally given the formula Ni₃(Al, Ti). However, both the nickel and the aluminium and titanium can be substituted by other elements.

The present inventors found that alloy 263, Haynes® 282® and Inconel® 740 all developed as wrought alloys were the most promising candidates particularly because of their high stress rupture strength as shown in Figure 1. However, alloy 263 suffers from microstructural instability upon service aging by the precipitation of eta (**η**) phase (Ni₃Ti), which can have a detrimental effect on creep strength. Haynes® 282® is the stronger of the three alloys, but the level of Al and Ti was the highest (Al+Ti >3.5%), and so the potential for oxidation of these elements during pouring in air was significantly increased. This could potentially lead to many more oxide inclusion defects within the casting. It was also known that during trials of casting alloy 282, the heavy section microstructural integrity was poor, which lead to volumetric cracking far worse than observed in either alloy 263 or Inconel® 740.

Inconel® 740 was developed as a cast and wrought product for advanced ultra super critical boiler tubes. In the wrought process the alloy is cast as a billet and then subjected to mechanical deformation to form it roughly into the desired shape. Final machining steps are then taken to achieve the desired shape.

The composition of Inconel® 740 was derived from the aero alloy Nimonic 263, and is age hardenable at around 800°C. The nominal compositions of these two are shown in table 2.

**Table 2: Nominal Alloy 740 Composition from Special Metals Datasheet (Inconel^{®} 740)**

| Alloy | Fe | C | Si | Mn | Ni | Cr | Mo | Nb | Co | Al | Ti |
|---|---|---|---|---|---|---|---|---|---|---|---|
| 263 | 0.7 | 0.06 | 0.10 | 0.30 | Bal | 20.0 | 6.0 | Residual | 20.0 | 0.4 | 2.2 |
| 740 | 0.7 | 0.03 | 0.50 | 0.30 | Bal | 25.0 | 0.50 | 2.0 | 20.0 | 0.9 | 1.8 |

Unfortunately, the original Inconel® 740 composition seems to have been prone to welding micro fissuring of heavy section pipe work, the formation of detrimental "G" phase and is still prone to precipitation of Eta (**η**) phase, but to a lesser extent than alloy 263.

J. M. Sanders et al (2009) disclose a filler metal alloy for welding Inconel alloy 740, consisting of (in mass %) 24.13% Cr, 19.76% Co, 1.26% Al, 1.31% Ti, 0.55% Fe, 0.031% C, 019% Si, 0.37% Mn, 0.061% Cu, 0.58% Mo, 0.93% Nb, 0.001% B, 0.003% Zr, 0.005% V, less than 0.001% Ta, 0.004% P, 0.002% W, less than 0.001% N, and the balance Ni plus impurities ("Elimination of Fissures in Thick Section INCONEL Alloy 740 Welds", Technical paper BR-1827 Babcock & Wilcox Power Generation Group Inc).

To solve this problem, the Inconel® 740 alloy composition was changed to produce an alloy called 740H and presented at the EPRI "Sixth International conference on advances in material technology for fossil power plants" - Oct 2010 in a paper called *"Optimization of INCONEL*® *alloy 740 for Advanced Ultra Supercritical Boilers".* This paper describes the changes that Special Metals had carried out to the Inconel® 740 chemistry and is detailed in table 3 below. Note the changes in Si, Nb, Al and Ti composition.

**Table 3: Optimisation of Inconel® 740 for Advanced Ultra Supercritical Boilers**

| | Fe | C | Si | Mn | Ni | Cr | Mo | Nb | Co | Al | Ti |
|---|---|---|---|---|---|---|---|---|---|---|---|
| Alloy 740 | 0.7 | 0.03 | 0.50 | 0.30 | Bal | 25.0 | 0.50 | 2.0 | 20.0 | 0.9 | 1.8 |
| Alloy 740H | 0.7 | 0.03 | 0.15 | 0.30 | Bal | 25.0 | 0.50 | 1.5 | 20.0 | 1.35 | 1.35 |

The rational behind each elemental change is summarised as follows:
"G" Phase is a Si rich phase and therefore Si was reduced in the target specification to retard its formation. Reduced Nb content limited the tendency of the material's susceptibility to liquation cracks at the heat affected zone. The Al: Ti ratio was increased to enhance the stability of Gamma Prime (γ') and this is the prime reason for fissuring being prevented due to the more stable aged matrix, while reducing Ti would decrease the material's ability to produce acicular Eta (**η**) phase in service at 725°C.

The present inventors found that if the standard wrought alloy 740 or 740H chemistry is used in a casting, cracks form after heat treatment which causes NDE failures and scrap castings.

Upon SEM investigation the cracks were found to be volumetric in nature and seem to be propagated from the inter-granular regions of the alloy. At these inter-granular grain boundary regions, Nb rich MX particles exist which themselves crack during heat treatment. These particles are the reason for the loss of boundary cohesion which is the cause of the cracking, during the stresses set up within the material during heat treatment. Additionally, vacancies formed by partial dissolution of the Nb MX along the grain boundaries after solution treatment, produced propagation sites for cracking at the grain boundaries.

Figure 2 shows an SEM micrograph of a grain boundary in a cast Inconel 740H, after a homogenising heat treatment at 1100°C. As can be seen, two grain boundary phases are present. The inventors have found these to be a Ti rich MX phase and a Nb rich MX phase. As can be seen from the SEM micrograph, the Nb rich MX phase is cracked. It is thought that this is due to the difference in coefficient of thermal expansion between the matrix and Nb rich MX phase.

A series of heat treatment trials were made to determine the stage at which the cracking of the precipitates takes place, and to establish if the cracking can be avoided by adjusting ramp and cooling rates. These are shown in table 4.

**Table 4**

| Condition | Comments |
|---|---|
| Homogenise @ 1100°C + Quench | Fast cooling rate |
| Homogenise @ 1100°C + Air Cool | Slower Cooling |
| Homogenise @ 1100°C + Furnace Cool | Slowest Cooling |
| Homogenise @ 1100°C + Solution 1200°C + Air Cool | - |
| Homogenise @ 1100°C + Solution 1150°C | Ramp 6°C/min - Cooling 1°C/min |
| Homogenise @ 1100°C + Solution 1150°C + 1200°C | - |

In all conditions in table 4 the Nb rich MX precipitates were present and most were cracked.

Differential scanning calorimeter (DSC) curves show that the dissolution temperature of Nb rich MX was likely to be in the order of 1350°C. However, the melting point of the alloy is around 1400°C. Therefore, it seems to be almost impossible to dissolve the blocky Nb rich MX to eliminate cracking through the MX once it has been formed after solidification in the wrought Inconel® 740 and Inconel® 740H compositions.

Therefore, the inventors concluded that it is not possible to remove the Nb rich MX particles from the cast alloy Inconel® 740H by heat treatment alone, or to prevent the cracking by reduction of ramp and cooling rates as the MX precipitates are present immediately after the liquid is solidified. By experimentation and thermal analysis, the dissolution temperature of the Nb rich MX was found to be 1350°C. This dissolution temperature is too close to the melting point of the alloy for it to be utilised.

On the basis of the above, the inventors considered whether the composition of the alloy could be altered in order to reduce the formation of the Nb MX carbide. For a wrought alloy grain size control is possible in that during the wrought process recrystalisation can be achieved. By pinning the grain boundaries using carbides and other phases it is possible to maintain a small grain size. The inventors realised that, for a cast product, such grain size control is not achievable because recrystalisation is not promoted through mechanical deformation. So loss of the Nb MX and a potentially lower M₂₃C₆ phase might reduce grain boundary cohesion and some γ' phase fraction, but for a cast product the elimination of cracking is more important.

The present inventors used a thermodynamic model to calculate the equilibrium fraction of phases and individual element partitioning behaviour as a function of temperature.

The thermodynamic model calculates the equilibrium fraction of phases and individual element partitioning behaviour as a function of temperature when presented with bulk alloy element concentrations. The thermodynamic model contains mathematical algorithms which are used to determine the alloy phase characteristics. The mathematical algorithms use a database containing thermodynamic data for the alloy system of interest. The database contains essential technical data such as enthalpies of formation, entropy, chemical potentials, interaction coefficients, heat capacity and crystal structures. The thermodynamic calculations are based upon the minimisation of the Gibbs free energy.

Figure 3 shows the equilibrium phase diagram for Inconel® 740 with a composition as in table 5 (a composition near to that of the nominal composition of Inconel® 740) and Figure 4 shows the expanded equilibrium phase diagram to highlight the MX, **η** and M₂₃C₆ phases.

**Table 5: Composition for Equilibrium Calculation shown in Figures: 3 and 4**

| C | Ni | Cr | Mo | Nb | N | Ti | Co | B | Al |
|---|---|---|---|---|---|---|---|---|---|
| 0.04 | 51.3 | 24.62 | 0.54 | 1.31 | 0.023 | 1.36 | 19.57 | 0.0025 | 1.22 |

As can be seen, at high temperature (where equilibrium is more likely to be achieved) **η** and MX phases are in equilibrium. On cooling from these temperatures these phases may remain or precipitate after long term aging.

Table 6 shows how the composition of Inconel® 740 was changed by the present inventors. The new alloys, designed for producing products by casting, have a number of significant chemistry differences over the conventional wrought compositions which makes the alloy far more castable.

**Table 6: Standard Nominal Composition for Alloy 740H and nominal alloys of the invention**

| | C | Si | Mn | Ni | Cr | Mo | Nb | Ta | Al | Ti | Al+Ti | Fe | Co |
|---|---|---|---|---|---|---|---|---|---|---|---|---|---|
| Alloy 740H | 0.03 | 015 | 0.30 | Bal | 25.0 | 0.50 | 1.5 | - | 1.35 | 135 | - | 0.7 | 20.0 |
| Proposed New Nominal Composition 1 | 0015 ↓ | 0.15 | 030 | Bal | 25.0 | 0.50 | 0.25↓ | - | 135 | 1.35 | - | 0.7 | 20.0 |
| Proposed New Nominal Composition 2 | 0.015↓ | 0.20↑ | 0.30 | Bal | 25.0 | 0.25↓ | 0.25↓ | 0.15↑ | 1.45↑ | 1.45↑ | ≥2.8↑ | 0.7 | 20.0 |

Figures 3 and 4), except Eta phase, which is brittle and causes cracks and/or loss in creep strength in service, is eliminated. As shown below, the desirable properties are also present in the inventive alloy for carbon content up to 0.020% and Nb content up to 0.50%. Additional benefits from the Nb reduction:
a) The alloy is less prone to segregation in heavy sections, as Nb is an element which has a high potential for segregation. This is shown in Figure 14 which is a Scheil Calculation showing non equilibrium segregation tendency for cast alloy 740.
b) The reduction of Nb lowers the solubility of Nitrogen in the air melted product, allowing for lower nitrogen levels to be achieved than with the standard product without specialised processes.

Figure 5 is the equilibrium phase diagram of the new nominal alloy composition 1 of table 6 and shows that the major phase thermodynamic predictions for the alloy are similar to alloy 740H, except that Eta phase is completely removed.

Figure 6 uses the same thermodynamic model to predict the composition of the MX phase in the alloy of the present invention. The composition of MX of the alloy of the present invention is different from that of standard Inconel 740H®. The alloy of the present invention has a Nb mass fraction increase of <0.01 above 900°C, and the Ti mass fraction is almost constant from 300 to melting point. Therefore, the predicted total mass fraction of MX is dramatically reduced.

Eta phase is deleterious, and is reduced in the cast alloy compared to in 740H further by the reduction of Nb.

Due to the reduction in Nb concentration, gamma Prime (γ') fraction is depressed in the alloy of the present invention compared to the case where the Nb content is higher such as in conventional wrought alloy. Nb substitutes for Al in (γ')(Ni₃Al), as does Ti. The wrought alloy 740 and 740H contain around 21% gamma prime (γ'). At this level of precipitation, in conjunction with high levels of MX precipitation, the inventors discovered that in the casting alloy room temperature ductility was very low. This is an important factor to consider when a plant in which the alloy is used is thermally cycled during shutdown and start up, and when in service repairs are required e.g. by welding. Therefore, the gamma prime (γ') is preferably increased in the inventive alloy to a level in which ductility is balanced with ultimate creep strength.

In a preferred embodiment, the amount of gamma prime (γ') is increased by ensuring that the total mass % of aluminium and titanium is greater than or equal to 2.8 mass %, preferably 2.9 mass % and/or by ensuring that the total amount of Ta is between 0.13 and 0.17 mass % and/or by having the amount of Nb being present in an amount of between 0.23 and 0.27 mass % and/or by increasing the amount of Mo to between 0.23 mass % and 0.27 mass %.

The alloy of the present invention consists of an alloy consisting of, in mass %, 24.0-26.0% Cr, 19.0-22.0% Co, 1.00-1.60% Al, 1.00-1.60% Ti, up to 1.50% Fe, up to 0.020% C, up to 0.40% Si, up to 0.50% Mn, up to 0.50% Cu, up to 0.50% Mo, up to 0.50% Nb, up to 0.005% B, up to 0.03% Zr, up to 0.10% V, up to 0.02% Mg, up to 0.25% Ta, up to 0.010% S, up to 0.015% P, up to 0.20% W, up to 0.02% Ca, up to 0.05% N, up to 80 ppm Zn, up to 60 ppm Sn, up to 20 ppm Pb, and the balance Ni plus trace additions and impurities.

The term "consisting of" is used herein to indicate that 100% of the composition is being referred to and the presence of additional components is excluded so that the percentages add up to 100%.

The rational of the inventive composition is defined below. All amounts are mass % unless otherwise stated:

### Nickel: Balance

This is the matrix element as it forms the balance of the material chemistry, and has good solubility for a large variety of secondary elements and consequently can be easily alloyed. The FCC nickel lattice is compatible with both solid solution and precipitation strengthening mechanisms.

### Chromium: 24.0-26.0 Mass %, preferably 24.5 to 25.0 mass %

Chromium provides crucial corrosion resistance to the alloy by rapidly forming a surface (Cr₂O₃) layer under hot corrosion, which effectively shields the underlying alloy from excessive corrosion attack. Chromium also assists the formation of a surface alumina layer at low temperature, which further enhances the corrosion resistance of the alloy. In conjunction with Mg (up to 0.02%) and Si (up to 0.4%), the protective nature of the scale is even more enhanced and made effective to higher temperatures. The function of these minor elements is to enhance scale adhesion, scale density and resistance of the scale to decomposition.

Chromium has a mild solid solution strengthening effect on the matrix due to atomic parameter mismatch with Ni.

The minimum level of Cr is chosen to assure α-chromia scale formation at an elevated temperature. This level of Cr is about 24.0% preferably 24.5%. Slightly higher Cr levels accelerate α-chromia formation but do not change the nature of the scale. The maximum Cr level is determined by alloy stability. This maximum level of Cr was found to be about 26.0%, or better 25.0%.

### Colbalt: 19.0 to 22.0 mass %, preferably 19.5 to 20.5 mass %

The main purpose of adding Co is indirectly to increase the solidus temperature and subsequently the operating temperature of the alloy by improving solubility of the γ' precipitates. This increase raises the y volume fraction of the alloy and exerts an extra strengthening effect so amounts of greater than 19.0% are used, desirably greater than 19.5%.

The similar atomic size of cobalt with that of nickel limits its solid solution strengthening effect to the matrix, and due to cost the amount is limited to 22.0% or less, desirably 20.5% or less.

### Aluminium: 1.00 to 1.60 mass %, preferably 1.20 to 1.55 mass %, more preferably 1.40 to 1.55 mass %.

Aluminium is a major alloying element which partitions to the y precipitates. As a principal y forming element, it has direct influence on y volume fraction and consequently precipitation strengthening of the alloy so Al is present in an amount of at least 1.00 mass % desirably at least 1.20 mass %, more desirably at least 1.40 mass %.

Aluminium provides corrosion resistance to the alloy by forming a protective alumina (Al₂O₃) surface layer under hot corrosion. Excessive amounts of aluminium can reduce the ductility of the alloy so its amount is limited to 1.60 mass % or less, desirably 1.55 mass % or less.

### Titanium: 1.00 to 1.60 mass %, preferably 1.20 to 1.55 mass %, more preferably 1.40 to 1.55 mass %

Titanium is another major y forming element and it also tends to partition to the γ' phase so Ti is present in an amount of at least 1.00%, desirably at least 1.20%, more desirably at least 1.40%.

Ti in amounts in excess of 1.60% is prone in internal oxidation leading to reduced matrix ductility. Preferably Ti is present less than 1.55%.

Titanium shares similar precipitation strengthening effects as aluminium.

To further compensate for the reduction in Gamma Prime (γ') fraction by reduced Nb content, Al and Ti mass% are increased in the new alloy. Table 13 shows the effect of increasing Al + Ti mass % on estimated Gamma Prime (γ') fraction with balance chemistry as detailed in the proposed new nominal composition. G130 as Table 14. Desirably the mass % of Al + Ti is greater than or equal to 2.8 mass %, more desirably greater than or equal to 2.9 mass % or even greater than or equal to 3.0 mass %. In order to reduce the chance of oxidation during pouring in air, Al + Ti mass % is preferably kept below 3.15 mass % or more preferably less than 3.05 mass %.

### Niobium: 0.00 to 0.50 mass %, preferably 0.20 to 0.30 mass %, even more preferably 0.23 mass % to 0.27 mass %.

Niobium promotes y phase formation, but to a lesser extent than that of Al and Ti. The invention reduces the Nb level in the alloy to 0.50% or less or of less than 0.50% or preferably less than 0.40%. The presence of Nb leads to an increase in the volume fraction of γ' and so can be desirable at a level of 0.15% or more, more desirably at a level of at least 0.20 mass % or even at least 0.23 mass %.

The major benefit of reduced Nb is to prevent the precipitation of Nb rich MX (NbC). Another benefit is to reduce the tendency of Eta phase to form. Also Nb has a high tendency to segregate in heavy sectioned castings and limiting its concentration helps to reduce this tendency. In the invention amounts Nb of up to 0.30 mass % give a desirable small increase in gamma prime y volume fraction, without the formation of Nb rich MX or tendency for deleterious Eta(η) phase precipitation during service. However, a maximum amount of Nb of up to 0.49% or of up to 0.40%, more preferably 0.30% and most preferably up to 0.27 mass % is preferred to keep any chance of precipitation of MX low.

### Carbon: 0.000 to 0.020 mass %, preferably 0.005 to 0.015 mass %

Carbon is an alloying element which partitions the grain boundary regions. Its major function is to form a variety of carbides with other alloying elements and to provide increased grain boundary cohesion. Carbides predicted in the alloy of the invention are M₂₃C₆ and MX. Carbon also has a moderate solution strengthening when dispersed within the matrix.

An upper limit of 0.020 mass % limits the formation of Nb rich Mx, especially when Niobium is also reduced. The inventors found that levels of carbon above 0.02% will cause unacceptable levels of Nb MX within the casting, especially within section sizes >100mm. Preferably carbon is present in an amount of at least 0.005 mass % so as to achieve some grain boundary carbides and thereby increase grain boundary cohesion and to provide some solid solution strengthening when dispersed in the matrix. Preferably carbon is present at an amount of 0.015 mass % or less so as to avoid excessive carbide precipitation at the grain boundaries.

### Boron: 0.000 to 0.005 mass % and Zirconium 0.000 to 0.03 mass %

Boron and Zr can be added to inhibit carbide coarsening which consequently increases grain boundary strength. Creep strength and ductility are increased by the addition of these elements. Addition of Boron improves the resistance to grain boundary sliding.

### Manganese: 0.00 to 0.50 mass %, preferably 0.15 to 0.45 mass %

Manganese improves the weldability of the alloy by reducing its freezing range. So Mn is present up to 0.50 mass %, preferably at least 0.15 mass %. However, manganese reduces protective scale integrity so is preferably present in a maximum amount of 0.45 mass % or less.

### Silicon: 0.00 to 0.40 mass %, preferably 0.10 to 0.25 mass %

Silicon can control the morphology of carbides and can be beneficial for corrosion resistance. If Si levels are too high, then this can promote G phase formation.

Additionally, excessive amounts of Si can contribute to loss of ductility, toughness and workability. Therefore, Si is preferably present up to 0.40 mass % to take advantage of the morphological and carbide content control whilst limiting the loss of ductility, toughness and workability. A preferred range is 0.10 to 0.25 mass %.

### Molybdenum: 0.00 to 0.50 mass %, preferably 0.20 to 0.30 mass %, more preferably 0.23 to 0.27 mass %.

This invention limits the Mo content to 0.50%, due to its segregation tendency, and ability to form Mo rich precipitates (Carbides). Mo contributes to solid solution strengthening of the matrix. Mo is predominantly distributed within the gamma (γ) matrix, M₂₃C₆ and gamma prime. Mo contributes to solid solution strengthening of the gamma matrix, and a slight increase in gamma prime and is therefore preferably added within the range of 0.20 to 0.30 mass %, more preferably 0.23% to 0.28 mass %, ideally at 0.25 mass %, and compensates to overcome the strength lost by the removal of Nb. Figure 16 shows the predicted small, but beneficial effect of Mo on increase in gamma prime (γ') mass %.

This additional limit on elements which segregate in the casting alloy is of more importance compared with the wrought alloy, as the casting cannot be homogenised to the same extent as a wrought alloy.

### Nitrogen: 0.00 to 0.05 mass %, preferably 0.03 mass % max.

As Titanium is the most prominent nitride former, it readily combines with nitrogen to form MX. By keeping residual nitrogen to a minimum the formation of unnecessary MX, which will have a depletion effect on gamma prime y mass fraction, is prevented.

Sulphur and Phosphorous are undesirable trace elements and partition to the grain boundaries of the Ni Alloy. Therefore, these elements are desirably controlled to low levels so as not to effect grain boundary strength.

Sulphur is desirably controlled to 0.010 mass % maximum but preferably 0.005% max, but ideally less than or equal to 0.001 mass %, and Phosphorous to 0.015 mass % max, but preferably 0.010%max.

Zinc, Tin and Lead are low melting point constituents and are considered tramp elements in Ni alloys as their presence can effect grain boundary cohesion. Desirably they are limited to 80 ppm Zn, 60 ppm Sn and 20 ppm Pb, more desirably they are limited to 30 ppm Zn, 50 ppm Sn and 10 ppm Pb.

Tantalum is a carbide former in Ni alloys, and is desirably limited to 0.25 max %.. . The inventors realised that Tantalum increases Gamma Prime (γ') mass fraction by 0.2% with addition of 0.15 mass %, according to simulations performed. It can also be seen from equilibrium calculations that Ta only distributes in Gamma (γ) and Gamma Prime (γ'). Therefore, adding of Ta will have no effect on increasing undesirable MX. Therefore, in the inventive alloy preferably Ta is present at a level of 0.10-0.20 mass %, more desirably 0.13-0.17 mass %. Figure 15 shows the effect of Tantalum on gamma prime (γ') mass %.

Copper is not an intentional addition in the invention and is considered residual and therefore is limited to 0.50 mass % but preferably 0.10 mass %.

Iron has some solid solution strengthening properties, but is limited to 1.50% mass, preferably to 1.00% in this invention, and more preferably less than 0.80% and is considered residual.

Vanadium and Tungsten are not intentionally added in the invention, and are limited to the following values W: 0.20 mass % max, desirably 0.05 mass % max, Vanadium: 0.10 mass % max, desirably 0.05 mass % max.

Magnesium can be used as a deoxidiser or desulphuriser and Mg levels can be tolerated within the alloy up to 0.02 mass %, however, in the casting alloy should be preferably limited to 0.01 mass % due its tendency to cause oxide films when cast in air.

Calcium can be added as a desulphuriser and deoxidiser, and in this respect can be allowed up to 0.02 mass %, desirably only up to 0.01 mass %.

### List of Main Phases Present in the Cast Alloy during Characterisation:

### Matrix: Gamma (γ)

The alloy matrix consists of γ (gamma) with up to 20% γ'.

### Gamma Prime (γ')

The γ' phase provides strong precipitation strengthening to the alloy.

### MX

The reduction of Nb content to less than 0.50% or lower and lowering carbon content, means that Nb rich MX will not be formed. Therefore, MX mass fraction will be lower than that of alloy 740 and 740H.

M₂₃C₆ is a Cr rich precipitate which usually forms along grain boundaries as in many other nickel-based superalloys. It precipitates as a function of lower temperature ageing.

Sigma: this phase is traditionally high in Cr content and is a low temperature phase. Sigma has not been detected in the invention in the solution treated and aged condition.

### M₃B₂: None detected.

For the foundry, successfully producing solid solution strengthened alloys as heavy section castings is now a commercial reality.

For the gamma prime (γ') strengthened alloys, as these alloys are relatively new, there is little experience world wide of casting these new materials, and there are no casting specifications available.

With these alloys special consideration are desirably be given to the following:
a) Melting Practice: Melting practices for Ni Alloys are different from conventional steel production in many ways. Specialised techniques can be used to prevent oxidation of volatile alloying elements. VOD, VODC or AOD melting is employed for the production of large components.
b) Pouring Technology: Ni Alloys that are alloyed with Titanium and Aluminium, and poured in air, are desirably poured with care to prevent oxidation defects on the surface of the castings.
c) Solidification: Ni alloy solidification characteristics are completely different from steels, and conventional methoding techniques are often not satisfactory alone in producing an acceptable quality casting. A process for casting nickel alloys which can be used with the alloy of the present invention is disclosed in WO 2009/130472.
d) Heat Treatment: The alloy of this invention is heat treated ideally by solution treatment, followed by cooling such as water quenching, air cooling or when sections sizes permit, still air cooling, or for certain applications "as cast" without heat treatment. Specialised homogenisation techniques can be employed for certain section sizes.

The present invention therefore provides a new alloy composition for a precipitation hardened super alloy which has high stress rupture strength at temperatures of above 700°C and which can be cast as castings. Therefore, the alloy of the present invention is ideal for use for manufacture of steam turbine casings, valves and (ancillary) valve components, or any other application where high temperature above 700°C, strength and corrosion resistance are desirable, using a cast process. In an embodiment, the alloy is used in valve or a valve component for operation between 500°C and 850°C, desirably between 650°C and 750°C. An (ancillary) valve component may be a component such as a bonnet, cover, bend or elbow, perhaps operating at high temperature within the power plant. The following tables 7 and 8 summarise the present invention.
Tramp Elements: (Maximum Values)
Zn: 80 ppm max, desirably 30ppm max; Sn: 60 ppm, desirably 50ppm max; Pb 20 ppm max, desirably 10ppm max

**Table 7: Inventive alloy:**

| | Fe | C | Si | Mn | Ni | Cr | Cu | Mo | Nb | Co | Al | Ti |
|---|---|---|---|---|---|---|---|---|---|---|---|---|
| Min | - | - | - | - | Bal | 24.0 | - | - | - | 19.0 | 1.00 | 1.00 |
| Max | 1.50 | 0.02 | 0.40 | 0.50 | | 26.0 | 0.50 | 0.50 | 0.50 | 22.0 | 1.60 | 1.60 |

| | B | Zr | V | Mg | Ta | W | Ca | S | P | N | | |
|---|---|---|---|---|---|---|---|---|---|---|---|---|
| Min | - | - | - | - | - | - | - | - | - | - | | |
| Max | 0.005 | 0.03 | 0.10 | 0.02 | 0.25 | 0.20 | 0.02 | 0.010 | 0.015 | 0.05 | | |

**Table 8: Preferred Ranges:**

| | Fe | C | Si | Mn | Ni | Cr | Cu | Mo | Nb | Ca | W |
|---|---|---|---|---|---|---|---|---|---|---|---|
| Min | - | 0.005 | 0.10 | 0.15 | Bal | 24.5 | - | 0.23 | 0.23 | - | - |
| Max | 0.80 | 0.015 | 0.25 | 0.45 | | 25.0 | 0.10 | 0.27 | 0.27 | 0.01 | 0.05 |

| | Ta | Co | Al | Ti | B | Zr | V | Mg | S | Al+Ti | |
|---|---|---|---|---|---|---|---|---|---|---|---|
| Min | 0.13 | 19.5 | 1.20 | 1.20 | - | - | - | - | | 2.8 | |
| Max | 0.17 | 20.5 | 1.55 | 1.55 | 0.005 | 0.025 | 0.05 | 0.01 | 0.001 | 3.05 | |

| | | | | | | | | | | | |
|---|---|---|---|---|---|---|---|---|---|---|---|
| *Sulphur: 0*.*005*%*max; Phosphorus: 0.010%max; Nitrogen: 0.03%max* | | | | | | | | | | | |

The invention is particularly applicable to one-off castings, such as those typically made using the sand moulding technique in which resin bonded particulate matter is used to make the mould. The particulate matter of a sand mould may be: sand, zircon, fused silica, alumina, magnesia, ceramic spheres or chromite for example or any combination thereof. For example, the alloy may be used for the manufacture by casting of high pressure steam turbine casings or valves for example used in a power station. For the latest advanced ultra super critical turbines the operating temperature of the component is over 700°C.

A series of thermodynamic predictions were made in which the nominal composition of all major elements are as in table 9. The results are in Figures 7 to 13 and tables 10 to 12.

| C | Ni | Cr | Mo | Nb | N | Ti | Co | B | Al |
|---|---|---|---|---|---|---|---|---|---|
| As Graphs | Balance | 24.62 | 0.54 | As Graphs | 0.023 | 1.36 | 19.57 | 0.0025 | 1.22 |

Figure 7 shows the variation in maximum γ' content between 400 and 1600°C on the x axis with variation in Nb content on the y axis at fixed carbon content of 0.015%. Whilst Inconel® 740 and 740H (assuming 0.015% carbon) have a γ' content of 21% and 19.7% respectively, the present invention with a Nb content of 0.5% has a γ' content of about 18% and at a Nb content of 0.25% a γ' content of about 17%. Thus, the alloy of the present invention will have good precipitation hardening properties.

Figure 8 shows the variation in maximum mass % of Nb MX phase on the y axis between 800 and 1350°C and mass % carbon on the x axis at fixed Nb content of 0.25%. As can be seen, at carbon content of less than 0.015%, the mass fraction of Nb MX is zero. This is the reason for the preferred upper level of C of 0.015% or less. However, even at carbon levels of up to 0.02% Nb MX is only present at less than 0.02 mass %. Figure 9 is similar to Figure 8 except that it shows the combined effect of Nb and C content by plotting Nb at the top of the graph on the x axis and C content on the bottom of the graph on the x axis. On the left hand side large amounts of Nb MX are present, but the level of Nb MX reduces as both Nb and C are reduced. At a Nb content of 0.43% and below and a C content of 0.015% and below, very little or no Nb MX is predicted to form.

The thermodynamic calculations show:
1) Eta phase is completely removed from the inventive alloy by decreasing carbon to 0.018% or lower and decreasing Nb to 0.54% or lower.
2) Nb MX is completely removed in the invention with carbon at 0.015% or lower and Nb at 0.43% or lower and gamma prime is predicted at 17%.

Figures 10 to 13 show the effect of reducing carbon content on Nb MX and Ti MX. All graphs assume a Nb content of 0.25% and the carbon content is 0.046%, 0.036%, 0.029% and 0.015% for Figures 10, 11, 12 and 13 respectively. As can be seen from the Figures, the amount of Nb in the MX phase (and amount of Nb MX as a fraction of total MX) reduces as the Nb content is reduced.

Both Nb and C are important in determining whether NbC will form, which has been shown to crack in large section castings. So keeping Nb and C content low, as in the present invention, is advantageous.

Tables 10 to 12 show the results of thermodynamic calculations based on the composition in table 9 (like Figures 7 to 13), with varying Nb and C content. The tables show the maximum amounts of Ti and Nb in any MX phase and the maximum amount of eta phase in a temperature range of 800 to 1350°C. The examples marked * fall outside the present invention.

**Table 10:**

| C | Nb | Gamma prime mass percentage (%) | Ti in MX | Nb in MX | Eta |
|---|---|---|---|---|---|
| *0.046 | *1.31 | 20 | 0.16 | 0.20 | Yes |
| *0.040 | *1.05 | 19 | 0.10 | 0.12 | Yes |
| *0.030 | *0.84 | 18 | 0.04 | 0.06 | Yes |
| 0.02 | *0.67 | 18 | <0.02 | 0.02 | Yes, very small |
| 0.018 | *0.54 | 18 | <0.02 | 0.02 | No |
| 0.015 | 0.43 | 17 | 0 | 0 | No |
| 0.012 | 0.34 | 17 | 0 | 0 | No |
| 0.009 | 0.27 | 17 | 0 | 0 | No |
| 0.007 | 0.22 | 17 | 0 | 0 | No |

**Table 11:**

| C | Nb | Gamma prime mass percentage (%) | Ti in MX | Nb in MX | Eta |
|---|---|---|---|---|---|
| *0.114 | 0.25 | 17 | 0.12 | 0.13 | No |
| *0.095 | 0.25 | 17 | 0.11 | 0.11 | No |
| *0.079 | 0.25 | 17 | 0.1 | 0.1 | No |
| *0.066 | 0.25 | 17 | 0.06 | 0.08 | No |
| *0.055 | 0.25 | 17 | 0.05 | 0.06 | No |
| *0.046 | 0.25 | 18 | 0.02 | 0.04 | No |
| *0.036 | 0.25 | 17 | No | 0.03 | No |
| *0.029 | 0.25 | 17 | 0 | 0.02 | No |
| *0.024 | 0.25 | 17 | 0 | 0.018 | No |
| 0.019 | 0.25 | 17 | 0 | 0.01 | No |
| 0.015 | 0.25 | 17 | 0 | 0 | No |
| 0.012 | 0.25 | 17 | 0 | 0 | No |
| 0.009 | 0.25 | 17 | 0 | 0 | No |

Therefore, because C has the most effect on the composition distribution of MX, lower C is desirably chosen.

**Table 12:**

| C | Nb | Gamma prime mass percentage (%) | Ti in MX | Nb in MX | Eta |
|---|---|---|---|---|---|
| 0.015 | 0.25 | 17 | 0 | 0 | 0 |
| 0.015 | 0.30 | 17 | 0 | 0 | 0 |
| 0.015 | 0.36 | 18 | 0 | 0 | 0 |
| 0.015 | 0.43 | 18 | 0 | 0 | 0 |
| 0.015 | *0.52 | 18 | 0 | 0 | 0 |
| 0.015 | *0.62 | 18 | 0 | 0 | little |
| 0.015 | *0.75 | 18 | 0 | 0 | yes |
| 0.015 | *0.89 | 18 | 0 | 0 | yes |
| 0.015 | *1.07 | 19 | 0 | <0.02 | Yes |
| 0.015 | *1.29 | 19 | 0 | <0.02 | yes |
| 0.015 | *1.55 | 20 | 0 | 0.02 | yes |
| 0.015 | *1.86 | 21 | 0 | 0.02 | Yes |

It can be seen that eta phase appears when Nb increases to 0.62 wt. %, and the percentage of gamma prime increases from 17 to 21% when Nb increases from 0.25 to 1.86 wt. %.

Therefore, Nb has the most effect on gamma prime and eta phase.

Eta phase is fully disappeared at 0.018% C and lower and 0.54% Nb and lower composition. The distribution lines of Ti and Nb are nearly flat at 0.015% C and lower and 0.43% Nb and lower composition. During the calculation, the fraction of gamma prime decrease from 20% to 17% as the content of Nb decreases.

Figures 7 to 13 and tables 10 to 12 show that C has more effect on MX than Nb and the more the C, the more NbC from the prediction. Nb also has an effect on eta phase and gamma prime, and the percentages of eta phase and gamma prime increase with increased Nb content. Therefore, keeping C at a low content (depending on practicalities) whilst at the same time selecting a suitable Nb content, results in sufficient gamma prime and no eta phase.

From Figures 7 to 13 and tables 10 to 12, a maximum amount of carbon of 0.02% or less and a maximum amount of Nb of 0.5% or less can be derived for eliminating eta phase and maintaining the amount of Nb MX to very low levels. At a Nb content of 0.25% or less or at a C content of 0.015% or less, the presence of eta and Nb MX is eliminated.

The inventors realised that a small increase in the fraction of γ' would increase strength of the alloy which could now be achieved without adverse impact on ductility due to reduced MX precipitation. In order to achieve an increase of the fraction of γ', the inventors investigated the effect of the total amount of Ti and Al in the alloy. Table 13 shows the results of equilibrium simulations at room temperature in which the amounts of Ti and Al are varied and the composition is otherwise equal to alloy G130 in Table 14.

**Table 13:**

| Al Mass % content | Ti Mass % content | Increased percentage (%) | Mass percentage of gamma prime (%) |
|---|---|---|---|
| Al:Ti=0.94 | | | |
| 1.3 | 1.39 | 0 | 17.7 |
| 1.36 | 1.46 | 5 | 18.6 |
| 1.43 | 1.52 | 10 | 19.6 |
| 1.49 | 1.59 | 15 | 20.5 |
| 1.56 | 1.66 | 20 | 21.5 |
| 1.62 | 1.73 | 25 | 22.4 (similar to 282M-22.5%) |
| 1.69 | 1.8 | 30 | 23.4 |
| 1.75 | 1.87 | 35 | 24.3 (similar to 282-24.6%) |
| 1.82 | 1.94 | 40 | 25.3 |
| 1.88 | 2.01 | 45 | 26.2 |
| 1.95 | 2.08 | 50 | 27.3 |

It can be seen that by increasing Al content to 1.43 mass % and Ti to 1.52 mass %, Gamma Prime (γ') can be increased by a factor of 10%.

On the basis of the results in Table 13, it is desirable that Al+Ti ≥ 2.8, more preferably ≥ 2.9 mass %, while maintaining a Ti % maximum of 1.6 mass % to prevent during long term service aging the precipitation of Eta (**η**) phase.

To additionally help offset the reduced predicted Gamma Prime (γ') fraction in the new alloy, 0.15 mass % Ta is added, with allowable levels up to 0.25 mass %. This has the effect of increasing Gamma Prime (γ') mass percentage as can be seen in Figure 15, where Gamma Prime (γ') mass percentage has been plotted against increasing Ta (mass %) while keeping Al, Ti, Nb, Mo and at the nominal proposed composition 1 as detailed in Table 6. Gamma Prime (γ') fraction will be increased by 0.2% with addition of 0.15 mass % Ta. From calculation Ta only distributes in Gamma (γ) and Gamma Prime (γ'). Therefore, adding of Ta will have no effect on increasing MX.

Table 14 shows the nominal composition of three test alloys in mass % falling within the scope of the invention. The right hand most column indicates the estimated mass fraction γ' for each alloy.

G130 melt was first produced and tested, the main goal being to ensure the microstructural integrity of the material from thin to thick section as would be required for a high integrity turbine component. Alloy G130 shows that lowering the carbon content and removing the Nb from alloy 740H reduces the MX precipitation to such an extent that intergranular cracking, and volumetric defects are eliminated.

G130 alloy has a lower strength than G130A and G130B thought to be caused by a lower y mass fraction. G130A and G130B address this without adding significant portions of MX into the alloy matrix (especially in heavy sections).

Increased γ' fraction over G130 was achieved by the introduction of nominally 0.25 mass%Nb, (G130A composition), and by additionally increasing the Al+Ti total content to ≥2.8mass%, and adding nominally 0.15mass% Ta (G130B composition). Figure 7 shows the effects of Nb on γ' mass fraction, Table 13 the effects of Al+Ti on γ' mass fraction, and Figure 15 the effects of Ta on y mass fraction. During all of the trials Mo was a purposeful addition and was added to a level of 0.25mass%. Figure 16 shows the effect of Mo on y mass fraction.

Table 15 summarises the main differences in composition and properties between G130, G130A and G130B.

**Table 15:**

| Alloy Name | Trial Heat Intentional Changes | Summary Results + Beneficial Effects on average Room Temperature Properties | | |
|---|---|---|---|---|
| G130 | Carbon reduced, Nb<0.05, Al+Ti=2.69 | Mx dramatically reduced | No inter granular cracking | No volumetric Defects |
| G130A | As G130 but with Nb increased to 0.23% | +7.2% avg increase in RT UTS | +14% avg RT Yield | No volumetric Defects |
| G130B | As G130A with Al+Ti>2.8% and 0.14% Ta Added | +5.2% avg increase in RT UTS | +6.2% avg RT Yield | - No volumetric Defects |
| TOTALS | | +12.4% room temp | +20.2% room | - |
| | | UTS | temp Yield | |

Tables 16 and 17 detail the room temperature and high temperature mechanical properties for alloys G130, G130A and G130B with sections of 100 mm and 200 mm thickness. The UTS, yield strength, elongation, reduction in area for tensile tests are given as well as Charpy Test results in the case of the room temperature test.

**Table 16:**

| Alloy Name | UTS (MPa) | | Yield (MPa) | | | |
|---|---|---|---|---|---|---|
| Section (½t) | 100mm | 200mm | 100mm | 200mm | | |
| G130 | 639 | 600 | 393 | 389 | | |
| G130A | 671 | 658 | 451 | 443 | | |
| G130B | 687 | 709 | 470 | 480 | | |

| | Elongation (%) | | R in A (%) | | Avg Impact Value Room Temp (J) | |
|---|---|---|---|---|---|---|
| Section (½t) | 100mm | 200mm | 100mm | 200mm | 100mm | 200mm |
| G130 | 74 | 25 | 51 | 29 | 200 | 221 |
| G130A | 50.2 | 39.8 | 37.3 | 40.1 | 160 | 167 |
| G130B | 24.7 | 33.1 | 40.7 | 45.8 | 127 | 122 |

**Table 17:**

| Alloy Name | UTS (MPa) 700°C | | Yield (MPa) 700°C | | Elongation (%) 700°C | | R in A (%) 700°C | |
|---|---|---|---|---|---|---|---|---|
| Section | 100 mm | 200 mm | 100 mm | 200 mm | 100 mm | 200 mm | 100 mm | 200 mm |
| G130 | 465 | - | 278 | - | 25 | - | - | - |
| G130A | 470 | 489 | 407 | 399 | 9.4 | 18.4 | 20.7 | 55.8 |
| G130B | 573 | 554 | 428 | 388 | 18.2 | 29.6 | 18.9 | 21.8 |

| Alloy Name | UTS (MPa) 800°C | | Yield (MPa) 800°C | | Elongation (%) 800°C | | | R in A (%) 800°C |
|---|---|---|---|---|---|---|---|---|
| Section | 100 mm | 200 mm | 100 mm | 200 mm | 100 mm | 200 mm | 100 mm | 200 mm |
| G130 | 420 | - | 263 | - | 20 | - | - | - |
| G130A | 401 | 409 | 343 | 387 | 4.5 | 5.4 | 12.1 | 10.0 |
| G130B | 438 | 440 | 325 | 356 | 15.6 | 10.6 | 47.9 | 21.7 |

As can be see, the mechanical properties of G130B are superior to those of G130A which are superior to those of G130.

Figure 17 shows the thick section tensile strength advantage of the G130B, G130A and G130 alloys over other precipitation hardened Ni alloys produced as castings. The inventive alloy has improved UTS at 200mm section tested over cast alloys 282, 263 and 740H, while the inventive alloys tested are comparable at 100mm section to the alloys 282, 263 and 740H. However, for the 263 and 282 alloys, their elongation and reduction in area properties are far inferior making the materials very difficult to process, weld repair, and fabricate and may mean that these materials have a maximum specified section size limit.

Figure 18 details the room temperature yield strength of the inventive alloys, which is comparable with other candidate A-USC cast alloys.

Alloy 263 is known as a candidate for 750°C A-USC application, although it can suffer from long term service instability. The material is generally known for it's good general ductility compared to other precipitation hardened Ni alloys and good weld ability characteristics. However, Figure 19 shows that when cast as a casting the heavy section ductility of the material is poor compared to the G130B alloy, while as Figure 18 shows, the room temperature strength of the inventive alloy is comparable or higher than alloy 263.

Figure 20 shows the stress rupture performance of alloys G130 and G130B compared to other cast Ni alloys after short term testing. It shows that alloy G130 performs better than solid solution strengthened alloy, but as expected lower strength than other precipitation strengthened alloys. However, alloy G130 is useable as it does not suffer from microstructural cracking in heavy section which is a problem with alloy 263, 740 and 282 and prevent their use as heavy section castings. G130 does also not suffer from the formation of detrimental eta phase in service which is a problem with standard composition alloy 740 and alloy 263. The results for G130B (preferred alloy range) in figure 20 show for higher stress rupture strength than G130, and test stress results are close to within scatter band for cast alloy 263. However, it should be noted, that the data for cast alloy 263, 740 and 282 are taken from very small 7kg castings, and will not represent stress rupture strength in a true thick section component. When 263, 740, and 282 were tested in larger test piece size, e.g. in castings over 500kg, most of the stress rupture samples broke early, or even on loading, due to very poor microstructural grain boundary integrity.

However, the results for G130 and G130B are from suitably large test material and, therefore, relate to true component properties. Additionally, no premature failures were experienced.

Figure 21 details short term stress rupture versus Larsen miller parameter for two alloys (G130 and G130B) within the scope of the invention and for differing section sizes. The graph shows that the A-USC target criteria of 80MPa at 700°C for 100,000hrs can be clearly met by all the material tested, and the G130B melt (preferred composition) where samples are still ongoing looks likely to achieve 80MPa at 750°C for 100,000hrs application.

Figure 22 is an SEM micrograph of a grain boundary of alloy G130B after casting and heat treatment showing that no MX carbide precipitates are present.

## Claims

1. An alloy consisting of, in mass %, 24.0-26.0% Cr, 19.0-22.0% Co, 1.00-1.60% Al, 1.00-1.60% Ti, up to 1.50% Fe, up to 0.020% C, up to 0.40% Si, up to 0.50% Mn, up to 0.50% Cu, up to 0.50% Mo, up to 0.50% Nb, up to 0.005% B, up to 0.03% Zr, up to 0.10% V, up to 0.02% Mg, up to 0.25% Ta, up to 0.010% S, up to 0.015% P, up to 0.20% W, up to 0.02% Ca, up to 0.05% N, up to 80 ppm Zn, up to 60 ppm Sn, up to 20 ppm Pb, and the balance Ni plus impurities.

2. The alloy of claim 1, consisting of less than 0.50% Nb or less than 0.49% Nb, preferably less than 0.40% Nb, and/or
consisting of up to 0.25% Nb, preferably of up to 0.15% Nb, or consisting of between 0.20-0.30% Nb, preferably 0.23-0.27% Nb.

3. The alloy of claims 1 to 2, consisting of up to 0.015% C, and/or
consisting of 0.005% or more C.

4. The alloy of any of claims 1 to 3, consisting of between 0.10-0.20% Ta, preferably 0.13-0.17% Ta.

5. The alloy of any of claims 1 to 4, consisting of at least 2.8 mass % Ti + Al, desirably at least 2.9 mass % Ti + Al, and/or
consisting of less than 3.15 mass % Ti + Al, desirably less than 3.05 mass % Ti + Al.

6. The alloy of any of claims 1 to 5, consisting of 1.40 to 1.55% Al, and/or consisting of 1.40 to 1.55% Ti.

7. The alloy of any of claims 1 to 6, consisting of between 0.20-0.30% Mo, preferably 0.23-0.27% Mo.

8. The alloy of any of claims 1 to 7, consisting of 0.10 to 0.25% Si, and/or consisting of 0.15 to 0.45% Mn, and/or
consisting of up to 0.10% Cu, and/or
consisting of up to 1.00% Fe, preferably up to 0.80% Fe and/or
including Mg.

9. The alloy of any of claims 1 to 8, consisting of 24.5 to 25.0% Cr and/or consisting of 19.5 to 20.5% Co.

10. The alloy of any of claims 1 to 9, consisting of up to 0.03% N, and/or
consisting of up to 0.005% S, more desirably 0.001 % S, and/or
consisting of up to 0.010% P, and/or
consisting of up to 0.01% Ca, and/or
consisting of up to 0.05% W, and/or
consisting of up to 0.05% V, and/or
consisting of up to 30 ppm Zn, up to 50 ppm Sn, up to 10 ppm Pb.

11. A cast product comprising the alloy of any of claims 1 to 10.

12. A steam or gas turbine casing or valve comprising the alloy of any of claims 1 to 10.

13. A valve or valve component comprising the alloy of any claims 1 to 10.

14. The steam or gas turbine casing, valve or valve component of claim 12 or 13,
wherein the component is a cast product.

15. The valve or valve component of claim 14, wherein the valve or valve component is for operation between 500°C and 850°C, desirably between 650°C and 750°C.

## Patentansprüche

1. Legierung, in Masseprozent bestehend aus 24,0-26,0% Cr, 19,0-22,0% Co, 1,00-1,60% Al, 1,00-1,60% Ti, bis zu 1,50% Fe, bis zu 0,020% C, bis zu 0,40% Si, bis zu 0,50% Mn, bis zu 0,50% Cu, bis zu 0,50% Mo, bis zu 0,50% Nb, bis zu 0,005% B, bis zu 0,03% Zr, bis zu 0,10% V, bis zu 0,02% Mg, bis zu 0,25% Ta, bis zu 0,010% S, bis zu 0,015% P, bis zu 0,20% W, bis zu 0,02% Ca, bis zu 0,05% N, bis zu 80 ppm Zn, bis zu 60 ppm Sn, bis zu 20 ppm Pb und der Rest Ni plus Vereinigungen.

2. Legierung nach Anspruch 1, bestehend aus weniger als 0,50% Nb oder weniger als 0,49% Nb, bevorzugt weniger als 0,40% Nb und/oder
bestehend aus bis zu 0,25% Nb, bevorzugt bis zu 0,15% Nb oder
bestehend aus zwischen 0,20-0,30% Nb, bevorzugt 0,23-0,27% Nb.

3. Legierung nach den Ansprüchen 1 bis 2, bestehend aus bis zu 0,015% C und/oder bestehend aus 0,005% oder mehr C.

4. Legierung nach einem der Ansprüche 1 bis 3, bestehend aus zwischen 0,10-0,20% Ta, bevorzugt 0,13-0,17% Ta.

5. Legierung nach einem der Ansprüche 1 bis 4, bestehend aus mindestens 2,8 Masseprozent Ti + Al, wünschenswerterweise mindestens 2,9 Masseprozent Ti + Al und/oder bestehend aus weniger als 3,15 Masseprozent Ti + Al, wünschenswerterweise weniger als 3,05 Masseprozent Ti + Al.

6. Legierung nach einem der Ansprüche 1 bis 5, bestehend aus 1,40 bis 1,55% Al und/oder bestehend aus 1,40 bis 1,55% Ti.

7. Legierung nach einem der Ansprüche 1 bis 6, bestehend aus zwischen 0,20-0,30% Mo, bevorzugt 0,23-0,27% Mo.

8. Legierung nach einem der Ansprüche 1 bis 7, bestehend aus 0,10 bis 0,25% Si und/oder bestehend aus 0,15 bis 0,45% Mn und/oder bestehend aus bis zu 0,10% Cu und/oder bestehend aus bis zu 1,00% Fe, bevorzugt bis zu 0,80% Fe und/oder Mg umfassend.

9. Legierung nach einem der Ansprüche 1 bis 8, bestehend aus 24,5 bis 25,0% Cr und/oder bestehend aus 19,5 bis 20,5% Co.

10. Legierung nach einem der Ansprüche 1 bis 9,
bestehend aus bis zu 0,03% N und/oder
bestehend aus bis zu 0,005% S, erwünschter 0,001% S und/oder bestehend aus bis zu 0,010% P und/oder
bestehend aus bis zu 0,01% Ca und/oder
bestehend aus bis zu 0,05% W und/oder
bestehend aus bis zu 0,05% V und/oder
bestehend aus bis zu 30 ppm Zn, bis zu 50 ppm Sn, bis zu 10 ppm Pb.

11. Gießprodukt, welches die Legierung nach einem der Ansprüche 1 bis 10 umfasst.

12. Dampf- oder Gasturbinengehäuse oder Ventil, welches die Legierung nach einem der Ansprüche 1 bis 10 umfasst.

13. Ventil oder Ventilkomponente, welche(s) die Legierung nach einem der Ansprüche 1 bis 10 umfasst.

14. Dampf- oder Gasturbinengehäuse, Ventil oder Ventilkomponente nach Anspruch 12 oder 13, wobei die Komponente ein Gießprodukt ist.

15. Ventil oder Ventilkomponente nach Anspruch 14, wobei das Ventil oder die Ventilkomponente für einen Einsatz zwischen 500°C und 850°C, wünschenswerterweise zwischen 650°C und 750°C, dient.

## Revendications

1. Alliage formé, en pourcentages massiques, de 24,0 à 26,0 % de chrome, 19,0 à 22,0 % de cobalt, 1,00 à 1,60 % d'aluminium, 1,00 à 1,60 % de titane, jusqu'à 1,50 % de fer, jusqu'à 0,020 % de carbone, jusqu'à 0,40 % de silicium, jusqu'à 0,50 % de manganèse, jusqu'à 0,50 % de cuivre, jusqu'à 0,50 % de molybdène, jusqu'à 0,50 % de niobium, jusqu'à 0,005 % de bore, jusqu'à 0,03 % de zirconium, jusqu'à 0,10 % de vanadium, jusqu'à 0,02 % de magnésium, jusqu'à 0,25 % de tantale, jusqu'à 0,010 % de soufre, jusqu'à 0,015 % de phosphore, jusqu'à 0,20 % de tungstène, jusqu'à 0,02 % de calcium, jusqu'à 0,05 % d'azote, jusqu'à 80 ppm de zinc, jusqu'à 60 ppm d'étain, et jusqu'à 20 ppm de plomb, et pour le complément, de nickel et d'impuretés.

2. Alliage conforme à la revendication 1, comprenant moins de 0,50 % de niobium ou moins de 0,49 % de niobium, de préférence moins de 0,40 % de niobium, et/ou comprenant jusqu'à 0,25 % de niobium et de préférence jusqu'à 0,15 % de niobium, ou comprenant de 0,20 % à 0,30 % de niobium, et de préférence de 0,23 % à 0,27 % de niobium.

3. Alliage conforme à la revendication 1 ou 2, comprenant jusqu'à 0,015 % de carbone, et/ou comprenant 0,005 % de carbone ou plus.

4. Alliage conforme à l'une des revendications 1 à 3, comprenant de 0,10 % à 0,20 % de tantale, de préférence de 0,13 % à 0,17 % de tantale.

5. Alliage conforme à l'une des revendications 1 à 4, comprenant au moins 2,8 % en masse, au total, de titane et d'aluminium, et de préférence, au moins 2,9 % en masse, au total, de titane et d'aluminium, et/ou comprenant moins de 3,15 % en masse, au total, de titane et d'aluminium, et de préférence, moins de 3,05 % en masse, au total, de titane et d'aluminium.

6. Alliage conforme à l'une des revendications 1 à 5, comprenant de 1,40 % à 1,55 % d'aluminium, et/ou comprenant de 1,40 % à 1,55 % de titane.

7. Alliage conforme à l'une des revendications 1 à 6, comprenant de 0,20 % à 0,30 % de molybdène, et de préférence de 0,23 % à 0,27 % de molybdène.

8. Alliage conforme à l'une des revendications 1 à 7,
- comprenant de 0,10 % à 0,25 % de silicium,
- et/ou comprenant de 0,15 % à 0,45 % de manganèse,
- et/ou comprenant jusqu'à 0,10 % de cuivre,
- et/ou comprenant jusqu'à 1,00 % de fer, de préférence jusqu'à 0,80 % de fer,
- et/ou comprenant du magnésium.

9. Alliage conforme à l'une des revendications 1 à 8, comprenant de 24,5 % à 25,0 % de chrome, et/ou comprenant de 19,5 % à 20,5 % de cobalt.

10. Alliage conforme à l'une des revendications 1 à 9,
- comprenant jusqu'à 0,03 % d'azote,
- et/ou comprenant jusqu'à 0,005 % de soufre, de préférence 0,001 % de soufre,
- et/ou comprenant jusqu'à 0,010 % de phosphore,
- et/ou comprenant jusqu'à 0,01 % de calcium,
- et/ou comprenant jusqu'à 0,05 % de tungstène,
- et/ou comprenant jusqu'à 0,05 % de vanadium,
- et/ou comprenant jusqu'à 30 ppm de zinc, jusqu'à 50 ppm d'étain, jusqu'à 10 ppm de plomb.

11. Produit de coulée comprenant un alliage conforme à l'une des revendications 1 à 10.

12. Enveloppe de turbine à vapeur ou à gaz, ou vanne, comprenant un alliage conforme à l'une des revendications 1 à 10.

13. Vanne ou composant de vanne, comprenant un alliage conforme à l'une des revendications 1 à 10.

14. Enveloppe de turbine à vapeur ou à gaz, vanne ou composant de vanne, conforme à la revendication 12 ou 13, laquelle pièce est un produit de coulée.

15. Vanne ou composant de vanne, conforme à la revendication 14, laquelle vanne ou lequel composant de vanne est conçu pour fonctionner entre 500 et 850 °C, et de préférence entre 650 et 750 °C.
